

# UNITED STATES PATENT OFFICE.

RUDOLPH FAUST, OF BROOKLYN, NEW YORK.

## STOVE POLISH.

1,403,758.

Specification of Letters Patent. Patented Jan. 17, 1922.

No Drawing.

Application filed May 11, 1921. Serial No. 468,770.

To all whom it may concern:

Be it known that I, RUDOLPH FAUST, a citizen of the United States, residing at the borough of Brooklyn, in the city of New York and State of New York, have invented certain new and useful Improvements in Stove Polish, of which the following is a specification.

This invention relates to polishes for stoves, and other similar metallic objects or articles; and it consists of certain ingredients mixed together in substantially the proportions hereinafter fully described and claimed.

15 The stove polish made according to this invention is formed of substantially:

10 pounds of plumbago,  
12 pounds of petrolatum, and  
1 pound of aluminum bronze powder.

20 These ingredients are mixed together, and about two ounces of oil of cloves is preferably mixed in with them.

The plumbago or graphite may have a percentage of black pigment, such as lamp black, mixed with it to strengthen its color if desired. The petrolatum is any kind of petroleum jelly, and vaseline may be used.

The aluminum bronze is a white metallic powder commercially known by that name, and its addition to the black coloring matter or plumbago greatly improves the appearance of the stove.

The oil of cloves is used to overcome any disagreeable oler in the mixture itself or while applying it. The polish is preferably applied to the stove while the stove is moderately hot, and by means of a soft cloth.

What I claim is:

1. A stove polish, comprising substantially ten pounds of black coloring matter, twelve pounds of petroleum jelly, and one pound of aluminum bronze powder.

2. A stove polish, comprising substantially ten pounds of black coloring matter, twelve pounds of petroleum jelly, one pound of aluminum bronze powder, and two ounces of perfume oil.

3. A stove polish, comprising substantially ten pounds of plumbago, twelve pounds of petrolatum, and one pound of aluminum bronze powder.

In testimony whereof I have affixed my signature.

RUDOLPH FAUST.